# EUROPEAN PATENT SPECIFICATION

(11) **EP 2 430 199 B1**
(45) Date of publication and mention of the grant of the patent: **29.05.2019**
(21) Application number: 10727754.3
(22) Date of filing: 16.04.2010
(51) Int. Cl.: C21D 8/02, C22C 38/04, C22C 38/12, C22C 38/14

(54) **METHOD FOR MANUFACTURING HOT ROLLED STEEL STRIP PRODUCT, AND HOT ROLLED STEEL STRIP PRODUCT**
VERFAHREN ZUR HERSTELLUNG EINES WARMGEWALZEN STAHLBANDES UND WARMGEWALZTES STAHLBAND PRODUKT
PROCÉDÉ DE LA FABRICATION D'UNE BANDE D'ACIER LAMINÉE À CHAUD ET LE PRODUIT DE LA BANDE D'ACIER LAMINÉE À CHAUD

(30) Priority: 11.05.2009 FI 20095528
(43) Date of publication of application: 21.03.2012
(73) Proprietor: Rautaruukki Oyj, 00620 Helsinki (FI)
(72) Inventor: LIIMATAINEN, Tommi, 92130 Raahe (FI); HEMMILÄ, Mikko, 86400 Vihanti (FI)
(74) Representative: Valea AB
(86) International application number: PCT/FI2010/050310
(87) International publication number: WO 2010/130871

(56) References cited:
- EP-A2- 1 319 725
- EP-B1- 1 375 694
- JP-A- 9 263 884
- US-A- 5 919 415
- US-A1- 2001 049 956
- US-A1- 2004 040 633

## Description

### BACKGROUND OF THE INVENTION

The invention relates to a method for manufacturing a hot rolled steel strip product having a wall thickness of 2 to 12 mm using steel whose composition in percentage by weight is

| | |
|---|---|
| C: | 0.04 - 0.08 |
| Si: | 0 - 0.5 |
| Mn: | 1.3 - 2.2 |
| Nb: | 0.04 - 0.09 |
| Ti: | 0.06 - 0.16 |
| N: | < 0.01 |
| P: | ≤ 0.03 |
| S: | < 0.015 |
| Al: | 0.01 - 0.15 |
| V: | ≤ 0.1 |
| Cr: | < 0.2 |
| Mo: | < 0.2 |
| Cu: | ≤ 0.5 |
| Ni: | ≤ 0.5 |

the rest consisting of iron and unavoidable impurities. Low carbon content is excellent for providing steel with good welding characteristics. Also the low carbon equivalent of steel has a positive effect to good weldability.

The invention further relates to a steel product with a wall thickness of 2 to 12 mm and a composition as described above.

EP 1319725 discloses a method for manufacturing a steel strip having the above composition. The strength of the steel strip thus manufactured is relatively high, its yield strength exceeding 690 MPa, combined with a relatively high percentage of elongation after fracture (12 to 21%). According to the publication these mechanical properties are arrived at by subjecting the steel to a two-step cooling. In the first cooling step an extremely fast cooling is carried out, the cooling rate being over 150°C/s after hot rolling, followed by a pause of 3 to 10 seconds without active cooling, after which a second cooling step is carried out to the coiling temperature of the steel strip to be manufactured, the temperature being chosen according to the desired strength. The recommended coiling temperature for yield strengths exceeding 690 MPa is 580°C. The high cooling rate of over 150°C/s at the first quenching step may be obtained only at low strip thicknesses, and the publication only discusses strip thicknesses lower than 4 mm. The cooling pause is meant to provide time for a phase change, during which the yield strength of the material in particular decreases and the yield strength/tensile strength value decreases compared with continued cooling. The publication does not disclose how a yield strength of over 690 MPa is obtained in the steel when the coiling temperature is below 580°C. The publication shows that the yield strength obtained in a coiling temperature of less than 580°C remains below 690 MPa.

US 2004/040633 A1 describes a hot strip or hot plate, and its production method. The steel is micro-alloyed and its disclosed chemical composition overlaps with the the composition claimed in the application. The method disclosed in US 2004/040633 A1 consists of casting the steel to form a raw material such as slabs, blooms, or thin slabs; heating to a temperature of 1300-1350°C; rough rolling at a degree of deformation of 36% to 43%; thermo-mechanically hot rolling at a finish roll temperature which exceeds the Ac3 temperature so as to form a hot strip; cooling at a cooling rate of at least 15C°/ s to a coiling temperature of 590-630°C.

Said two-step cooling is in practice more complicated to carry out than a one-step cooling and requires more complex production equipment. Moreover, the bendability of the steel strip obtained by two-step cooling is not particularly good, although the steel strip has relatively good values for percentage of elongation after fracture. Bendability means the ability of steel strip to bend to a small bending radius without surface damage emerging at the bending point. Two-step cooling has not succeeded in providing steel with particularly good impact strength values at low temperatures in combination with high strength.

### SUMMARY OF THE INVENTION

An object of the invention is to overcome said drawbacks of the prior art and to provide a method that is easy to implement for manufacturing strip steel product, typically a steel strip, of high strength and a particularly good bendability, the strip steel product having a chemical composition as mentioned above. To achieve this, the method of the invention is characterized by
- austenizing a work piece of steel at an austenizing temperature of 1200 to 1350°C;
- hot rolling the steel work piece in a pre-rolling step;
- rolling the pre-rolled steel work piece in a strip rolling mill so that a rolling temperature of 760 to 960°C for the work piece is achieved in the last pass; and
- direct quenching the steel strip after the last pass in the strip rolling mill by a single-step cooling at a cooling rate of 30 to 150°C/s to 300°C at the most, the direct quenching being carried out within 15s from the last pass.

The invention has surprisingly shown that said steel composition is capable of producing high-strength steel which also has good bendability. Also surprisingly, it was discovered that the strength of the steel is isotropic, i.e. its yield strength does not vary considerably irrespective of whether it is measured lengthwise or crosswise in relation to the rolling direction.

The direct quenching rate is preferably 120 °C/s at the most, because this enables to obtain a steel microstructure that provides the steel with particularly good mechanical properties, including good impact strength combined with good bendability.

Preferably, the end temperature of the direct quenching is 100°C at the most, because this enables to obtain a planar strip with also planar and even edges after the quenching.

Preferably, the steel strip is direct quenched directly to the coiling temperature and coiled.

The processing of the steel strip is preferably thermomechanical, and thus no tempering is carried out after the direct quenching. It has been observed that a steel product manufactured with the method has good mechanical properties although no tempering adding the costs is required on the product. Tempering does not significantly improve the mechanical properties of the product, and it complicates the process.

Preferred embodiments of the invention are disclosed in the accompanying claims 2 and 3.

The major advantages of the method of the invention are that it allows a steel product with good mechanical properties, including bendability, and a predetermined composition to be manufactured in a simple and economical manner and with simple equipment.

The invention further relates to a product manufactured in method steps of the invention.

The steel strip product of the invention having a wall thickness of 2 to 12 mm and composed in percentage by weight of

| | |
|---|---|
| C: | 0.04 - 0.08 |
| Si: | 0 - 0.5 |
| Mn: | 1.3 - 2.2 |
| Nb: | 0.04 - 0.09 |
| Ti: | 0.06 - 0.16 |
| N: | < 0.01 |
| P | ≤ 0.03 |
| S: | < 0.015 |
| Al: | 0.01 - 0.15 |
| V: | ≤ 0.1 |
| Cr: | < 0.2 |
| Mo: | < 0.2 |
| Cu: | ≤ 0.5 |
| Ni: | ≤ 0.5, |

the rest being iron and unavoidable impurities, is characterized in that the micro structure of the steel is substantially low carbon ferritic and/or low carbon bainitic, and contains high-carbon islands; that its yield strength is 650 - 800 MPa and percentage of elongation after fracture is at least 12%; that its yield ratio is 0.8-0.95; and that its structure is isotropic in the sense that its yield strength in the rolling direction differs 6.5% at the most from its yield strength in the direction that is transverse to the rolling direction.

High strength has been obtained although the microstructure of the steel mostly consists of a low carbon ferrite and/or bainite, without containing significant amounts of carbon-rich martensite or carbon-rich bainite. As recommended, the dominant phase consists of ferrite with an almost fully ferritic microstructure, as recommended, and small amounts of bainite and/or martensite and/or residue austenite in extremely small islands of enriched carbon content. A significant reason for the obtained high strength is the use of niobium and titanium as micro-alloy elements in the steel produced with the method. Both niobium and titanium must be used.

Preferred embodiments of the invention are disclosed in the accompanying claims 5 to 15.

The major advantages of the steel product of the invention are its excellent mechanical properties, including bendability and shear characteristics and impact strength values, in relation to its composition. The steel is also well applicable in arctic conditions. The steel of the invention is extremely useful due to its properties related to engineering works, because its weldability is good and its isotropic strength properties allow a very efficient optimization of its use. Moreover, the small bending radius particularly facilitates the work of bent product designers. The steel strip product of the invention is specifically well suited for use as strong structure steel.

### BRIEF DISCLOSURE OF THE FIGURES

In the following the invention will be disclosed in greater detail and with reference to the accompanying drawing in which
Figure 1 shows the method steps of the invention;
Figure 2 is a schematic view of a V-bending in bending tests;
Figure 3 illustrates an example of a successful bending test result;
Figure 4 illustrates an example of a failed bending test result;
Figure 5 presents transition curves for charpy-V obtained with the steel of the invention and a reference steel;
Figure 6 illustrates the connection between yield strength isotropy and strip rolling; and
Figure 7 illustrates the connection between yield strength isotropy and coiling temperature.

### DETAILED DISCLOSURE OF THE INVENTION

Figure 1 shows the method steps of the invention for producing a steel strip product with a wall thickness of 2 to 12mm. The manufacture starts with a work piece of steel whose composition in percentage by weight is

| | |
|---|---|
| C: | 0.04 - 0.08 |
| Si: | 0 - 0.5 |
| Mn: | 1.3 - 2.2 |
| Nb: | 0.04 - 0.09 |
| Ti: | 0.06 - 0.16 |
| N: | < 0.01 |
| P | ≤ 0.03 |
| S: | < 0.015 |
| Al: | 0.01 - 0.15 |
| V: | ≤ 0.1 |
| Cr: | < 0.2 |
| Mo: | < 0.2 |
| Cu: | ≤ 0.5 |
| Ni: | ≤ 0.5 |

and the rest iron and unavoidable impurities.

The steel has a low carbon content C of 0.04 to 0.08%, which is advantageous in view of the impact strength, bendability and weldability of the material.

Silicon, Si, may be used in an amount of 0 to 0.50% as a killing agent (in addition to aluminium) and for ferrite reinforcement. If a particularly good surface quality is to be aimed at, the silicon content must be limited to below 0.25%.

The alloying content of manganese, Mn, is 1.3 to 2.2%. Because of the low carbon content, steel is not prone to manganese and carbon segregation during casting, which enhances the homogeneity of the microstructure also at relatively high contents of Mn.

The steel of the invention may be cut into precisely dimensioned pieces both thermally (e.g. by laser and plasma) and mechanically. It has been observed that a piece with a relatively smooth cutting surface is obtained. This has an advantageous effect on fatigue strength. In addition, low carbon content prevents the cutting surface from becoming rough during thermal cutting and reduces maximum hardness, the cutting surface being less prone to brittle and crack during forming of the piece and in the conditions of use thereof. In mechanical cutting the cutting gap may be set at a value of 10 to 15% of the sheet thickness, the cutting result being still smooth and non-fractured and hence separate grinding of the cutting surface or thermal cutting is not needed, which significantly reduces working allowances and decreases the number of manufacturing steps, thereby enhancing the manufacturing process.

In order for a good impact strength and bendability to be achieved, the amounts of phosphor, P, (0.03% at the most) and sulphur, S, (0.015% at the most) present as impurities are to be restricted. The maximum amount of P is preferably 0.015% and that of S preferably 0.005%. Further, the properties may be improved, when necessary, by treatment with molten Ca or CaSi. As a killing agent, aluminium Al 0.01 - 0.15% is used. The amount of aluminium used is preferably 0.05% at the most.

The amount of nitrogen, N, used is 0.01% at the most, because when present in steel containing titanium, nitrogen forms hard titanium nitride particles that impair the bendability of the steel. The preferred amount of nitrogen used is 0.006% at the most.

The content of copper, Cu, is to be reduced to 0.3% at the most to ensure excellent surface quality for a hot-rolled strip. If the copper content exceeds 0.3%, it is recommended to alloy also nickel, Ni, in an amount equal to at least 0.25 times the Cu content. Although steel achieves its good properties also without copper, it may be used, when necessary, to slightly increase strength. The Cu content is 0.5% at the most. An alloy 0.3 to 0.5% of copper and at least 0.1% of nickel is preferably used particularly for thick strips of 8 to 12 mm, for example.

Even without copper in the alloy, Ni is restricted to 0.5% at the most. Although steel achieves its excellent strength properties also without the blending of Ni, it may slightly increase strength, when necessary.

Borium, B, is not alloyed at all, because it would unnecessarily increase hardening. Hence the borium content in the steel strip product of the invention is restricted to the impurity level, i.e. B < 0.0005%.

Titanium, T, may be alloyed to achieve a desired strength level. Typically 0.06 to 0.16%, although higher Ti levels could be used as well, but in that case its strength increasing effect is extremely small and may complicate the casting of the work piece. Lower Ti percentages are not used, because then high strength is difficult to obtain without using a more expensive alloying or increasing the carbon content to over 0.08%. Surprisingly the invention has shown that even at low temperatures, such as -40°C and -60°C, titanium does not lower significantly the impact strength of the basic agent, as shown by the measurement results of Table 3.

Chromium, Cr, and molybdene, Mo, do not need to be alloyed. They are elements that increase hardening and have a disadvantageous effect on weldability, at least in higher amounts. For this reason Cr is restricted to a maximum content of 0.2% and, similarly, Mo to a maximum content of 0.2%. The amount of chromium is preferably less than 0.1%.

Molybdene is most preferably allowed in an amount of 0.10%, and 0.2% at the most, because the mechanical properties of the steel of the invention are most preferably achieved by alloying titanium which provides more affordable alloying element costs than molybdene. Molybdene may even be harmful for strength in a direct quenched steel strip product of the invention. In any case, added molybdene does not significantly improve the strength of the steel strip product of the invention, when the product is produced by thermomechanical treatment.

Vanadine, V, does not need to be alloyed. In addition, it increases unnecessary hardening and has a disadvantageous effect on weldability at least in high concentrations. For this reason, V is restricted to a maximum content of 0.1%.

However, with low strip thicknesses t of 2 to 6 mm in particular, at high rolling forces, Nb and Ti concentrations are restricted as follows: Nb: 0.04 - 0.06% and Ti: 0.06 - 0.10% for reducing the rolling forces and, at the same time, a vanadium concentration V of 0.06 - 0.10% may be selected to obtain high strength.

With the low strip thicknesses t = 2 - 6 mm also silicon may be advantageously added in an amount of Si: 0.30 - 0.50% to increase strength, as shown in Table 1 of the tests run with an experimental composition E1.

According to a preferred embodiment of the invention the sum of the niobium, titanium and vanadium concentrations is greater than 0.15%, i.e. Ti + Nb + V > 0.15%, the steel strip product being applicable as a particularly strong structural steel.

At a lower carbon content limit in particular, the steel strip product of the invention is excellent to bend (fold) and to weld e.g. by autogenous high frequency (HF) welding into a tube or a tube beam. Manufacturing experiments have shown that the material suits excellently for producing HF-welded tube beams.

The work piece of steel is 210 mm thick, for example, and heated to an austenizing temperature of 1280°C, where it is kept for about 3 hours. Naturally the thickness of the steel work piece may differ from the one disclosed here and the austenizing temperature may be differently chosen, but a range of 1200 - 1350°C is recommended. If the austenizing temperature is below the lower limit given, there is a risk that the microalloying elements do not dissolve into the austenite, i.e. a homogenous austenite is not obtained. Most preferably the annealing time varies within a range of 2 to 4 hours.

The carbon equivalent C + Mn/6 + (Cr + Mo +V)/5 + Ni + Cu)/15 for steel is preferably not higher than 0.45, which guarantees a good weldability of the steel.

After austenizing, the steel work piece is hot-rolled at a temperature of 950 - 1250°C to a thickness which is typically 25 - 50 mm and then immediately transferred to a strip rolling mill to be rolled into a strip with a final thickness of 2 - 12 mm. The recommended final thickness of the steel strip is at least 4 mm. It also recommended that the final thickness does not exceed 10 mm.

The number of passes in the strip roll mill is typically 5 to 7. The last pass in the strip roll mill is carried out at a temperature range of 760 - 960°C, the recommendation being 780 - 850°C.

After the last pass the direct quenching of the steel strip starts within 15 seconds. At the start of the direct quenching the temperature of the steel strip must be at least 700°C. The direct quenching is carried out as a water quenching at a quenching rate of 30 - 150°C/s, the recommended upper limit being 120°C/s at the most. The direct quenching continues up to a temperature of 300°C at the most, the recommended temperature being 100°C. Immediately after the direct quenching the steel is coiled. Hence the coiling temperature may fall within a temperature range of 30 - 300°C. A recommended initial coiling temperature is 100°C at the most, because when steel is coiled at a temperature exceeding 100°C, a discontinuous steam cushion complicating the process may form onto the steel surface.

As a result of the thermomechanical treatment the microstructure of the steel becomes homogenous and consists of a dominant phase, which is preferably low carbon ferrite and/or low carbon bainite. The amount of the dominant phase is typically over 90%. In other words, extremely low amounts of high carbon bainite and/or residual austenite and/or martensite is present in extremely high carbon groups. The average grain size in the microstructure is small, preferably approximately 2 - 4 micrometers. It is also essential that the microstructure does not contain big grains in the first place and therefore the steel has particularly good bending characteristics taking into consideration the strength of the steel. The grain size must be as uniform and fine as possible, which is achieved by the method of the invention.

Tables 1 to 3 below provide examples of the concentrations and manufacturing parameters of the steel of the invention and of the strength and toughness values obtained with them. For the sake of comparison, Tables 2 and 3 also contain manufacturing parameters not belonging to the scope of the method of the invention, i.e. treatments not corresponding to the method of the invention. In Table 2 on the manufacturing parameters and in the table on the mechanical strength properties reference tests have been indicated with R.

A further topic of examination are the bending characteristics obtained with the treatments of the invention, these being compared with the bending characteristics obtained by manufacturing parameters remaining outside the scope of the method, see Tables 3 and 4, Steel B3Q23 (bending test a) according to the invention)and Steel A3M33 (bending test b) outside the invention).

Indication T_f in Table 2 denotes the temperature at the last rolling pass, indication T_c denoting the temperature at the start of the coiling, indication Th denoting the thickness of the steel strip and indication Wi denoting the width of the steel strip.

In the first column of Table 3 T denotes a sample whose strength and toughness have been determined in a direction transverse to the roll direction. Ending L denotes a sample whose strength and toughness have been determined in the rolling direction.

**TABLE 1. TEST COMPOSITION**

| anal | C | SI | MN | P | S | AL | NB | V | CU | CR | NI | N | MO | TI | CA | Ti+Nb+V | example |
|---|---|---|---|---|---|---|---|---|---|---|---|---|---|---|---|---|---|
| A1 | 0.049 | 0.23 | 1.99 | 0.008 | 0.003 | 0.03 | 0.08 | 0.01 | 0.03 | 0.04 | 0.04 | 0.005 | | 0.10 | | 0.20 | 1,2,3 |
| A2 | 0.049 | 0.19 | 1.92 | 0.007 | 0.003 | 0.03 | 0.09 | 0.01 | 0.04 | 0.04 | 0.05 | 0.005 | 0.01 | 0.10 | 0.003 | 0.19 | 10 |
| A3 | 0.049 | 0.19 | 1.89 | 0.009 | 0.002 | 0.03 | 0.08 | 0.01 | 0.01 | 0.03 | 0.05 | 0.006 | 0.00 | 0.10 | 0.003 | 0.19 | 9 |
| B2 | 0.056 | 021 | 1.81 | 0.007 | 0.003 | 0.03 | 0.09 | 0.01 | 0.04 | 0.04 | 0.05 | 0.007 | 0.01 | 0.11 | 0.003 | 0.21 | 5 |
| B3 | 0.058 | 021 | 1.76 | 0.008 | 0.004 | 0.03 | 0.08 | 0.01 | 0.03 | 0.04 | 0.05 | 0.004 | 0.01 | 0.11 | 0.002 | 0.19 | 6,9 |
| B4 | 0.064 | 021 | 1.78 | 0.011 | 0.001 | 0.03 | 0.09 | 0.01 | 0.04 | 0.06 | 0.06 | 0.009 | 0.01 | 0.11 | 0.003 | 0.20 | 4,10 |
| C1 | 0.053 | 0.18 | 1.78 | 0.008 | 0.004 | 0.03 | 0.06 | 0.00 | 0.03 | 0.05 | 0.05 | 0.008 | 0.01 | 0.14 | 0.003 | 0.19 | 8 |
| D1 | 0.057 | 0.17 | 1.65 | 0.008 | 0.003 | 0.03 | 0.04 | 0.01 | 0.03 | 0.03 | 0.04 | 0.005 | | 0.09 | | 0.14 | 7 |
| E1 | 0.079 | 0.39 | 1.43 | 0.011 | 0.003 | 0.03 | 0.05 | 0.08 | 0.04 | 0.06 | 0.06 | 0.007 | 0.01 | 0.06 | 0.002 | 0.20 | 11 |
| F1 | 0.061 | 0.23 | 1.79 | 0.008 | 0.001 | 0.04 | 0.08 | 0.01 | 0.40 | 0.07 | 0.20 | 0.007 | 0.01 | 0.12 | 0.002 | 0.22 | 12 |
| F2 | 0.058 | 0.20 | 1.90 | 0.007 | 0.002 | 0.03 | 0.08 | 0.01 | 0.40 | 0.06 | 021 | 0.006 | 0.02 | 0.12 | 0.002 | 0.21 | 12 |
| B5 | 0.06 | 021 | 1.81 | 0.009 | 0.004 | 0.03 | 0.08 | 0.01 | 0.04 | 0.07 | 0.08 | 0.007 | 0.02 | 0.11 | 0.002 | 0.20 | |

**TABLE 2. MANUFACTURING PARAMETERS.**

| sample | T_f | T_c | Th | Wi | example | | |
|---|---|---|---|---|---|---|---|
| A1M33 | 875 | 605 | 5 | 1260 | 1 | R | |
| A1M63 | 905 | 480 | 5 | 1260 | 2a | R | |
| A1Q61 | 920 | 250 | 5 | 1260 | 2b | | |
| A1M83 | 885 | 50 | 5 | 1260 | 3 | | |
| B2L13 | 910 | 360 | 10 | 1260 | 5 | R | |
| B3Q25 | 805 | 50 | 10 | 1270 | 6 | | |
| D1Q63 | 865 | 50 | 5 | 1500 | 7 | | |
| C1Q35 | 910 | 50 | 7.7 | 1355 | 8 | | |
| A3M33 | 890 | 615 | 10 | 1520 | 9 | R | bending b |
| B3Q23 | 830 | 50 | 10 | 1270 | 9 | | bending a |
| A2M33 | 895 | 605 | 8 | 1330 | 10 | R | transition curve 9c |
| B4Q23 | 835 | 50 | 8 | 1500 | 4.10 | | transition curve 9d |
| E1Q11 | 825 | 50 | 6 | 1500 | 11 | | |
| E1Q33 | 860 | 50 | 5 | 1500 | 11 | | |
| F1Q23 | 810 | 50 | 12 | 1500 | 12 | | |
| F2Q43 | 805 | 50 | 12 | 1250 | 12 | | |
| B5Q23 | 820 | 50 | 6 | 1500 | | | bending c |

**TABLE 3. STRENGTH AND TOUGHNESS PROPERTIES**

| sample | Th | RP02 | RM | RP02 difference (T-L)/L | A5 | ChV-20 | ChV-40 | ChV-60 | e.g. | | |
|---|---|---|---|---|---|---|---|---|---|---|---|
| | mm | MPa | MPa | % | % | J/cm2 | J/cm2 | J/cm2 | | | |
| **A1 M33T** | 5 | 829 | 873 | 9.8 % | 17.0 | | | | 1 | R | |
| **A1 M33L** | 5 | 748 | 833 | | 19.0 | 133 | 120 | 104 | 1 | R | |
| **A1 M63T** | 5 | 728 | 770 | 8.0 % | 16.0 | | | | 2a | R | |
| **A1 M63L** | 5 | 670 | 734 | | 18.0 | 245 | 216 | 187 | 2a | R | |
| **A1Q61T** | 5 | 747 | 850 | 7.0 % | 15.0 | | | | 2b | | |
| **A1Q61L** | 5 | 695 | 773 | | 15.0 | 211 | 205 | 189 | 2b | | |
| **A1 M83T** | 5 | 752 | 841 | 4.1 % | 15.0 | | | | 3 | | |
| **A1M83L** | 5 | 721 | 811 | | 16.0 | 216 | 195 | 187 | 3 | | |
| **B2L13T** | 10 | 734 | 812 | 10.4 % | 15.6 | | | | 5 | R | |
| **B2L13L** | 10 | 658 | 745 | | 17.6 | 221 | 234 | 185 | 5 | R | |
| **B3Q25T** | 10 | 736 | 835 | 0.0 % | 16.3 | | | | 6 | | |
| **B3Q25L** | 10 | 736 | 786 | | 17.5 | | | | 6 | | |
| **D1Q63T** | 5 | 678 | 794 | 6.3 % | 19.0 | | | | 7 | | |
| **D1Q63L** | 5 | 635 | 768 | | 20.0 | 235 | 221 | | 7 | | |
| **C1Q35pLA** | 7.7 | 737 | 852 | | 12.7 | 164 | 67 | 22 | 8 | | |
| **C1Q35pLB** | 7.7 | 708 | 815 | | 14.0 | | 140 | 88 | 8 | | |
| **A3M33L** | 10 | | 799 | | 19.2 | 84 | 73 | | 9 | R | bending b |
| **B3Q23T** | 10 | 717 | 810 | 1.7 % | 17.4 | | | | 9 | | bending a |
| **B3Q23L** | 10 | 705 | 786 | | 17.9 | 177 | 164 | 143 | 9 | | |
| **A2M33L** | 8 | 724 | 806 | | 18.0 | | 84 | | 10 | R | trans. curve 9c |
| **B4Q23T** | 8 | 745 | 837 | 0.4 % | 15.7 | | | 121 | 4.10 | | trans curve 9d |
| **B4Q23L** | 8 | 742 | 807 | | 17.1 | | 179 | 152 | 4.10 | | |
| **E1Q11T** | 6 | 737 | 855 | -1.6 % | 16.1 | | 165 | 143 | 11 | | |
| **E1Q11L** | 6 | 749 | 841 | | 16.4 | | 213 | | 11 | | |
| **E1Q33T** | 5 | 728 | 872 | 5.3 % | 16.1 | | 177 | | 11 | | |
| **E1 Q33L** | 5 | 691 | 845 | | 17.8 | | 223 | 157 | 11 | | |
| **F1Q23T** | 12 | 740 | 863 | 3.2 % | 16.2 | | | 127 | 12 | | |
| **F1Q23L** | 12 | 717 | 832 | | 18.1 | 227 | 209 | 198 | 12 | | |
| **F2Q43T** | 12 | 725 | 850 | 3.6 % | 16.2 | | | 122 | 12 | | |
| **F2Q43L** | 12 | 700 | 816 | | 17.9 | 215 | 213 | 182 | 12 | | |
| **B5Q23T** | 6 | 768 | 861 | 6.8 % | 15.7 | | 205 | 155 | | | bending c |
| **B5Q23L** | 6 | 719 | 827 | | 16.9 | | | 193 | | | bending c |

[Ex. A1Q61 and B5Q23] are comparative examples.

Tables 2 and 3 show that the impact strength values are good and the strength is isotropically high, when direct quenching is carried out to a low temperature (50°C).

As seen from Table 3, the yield strength of steels according to the invention is 635 - 829 MPa. The percentage of elongation after fracture A5 is at least 12% and typically at least 15%. The yield ratio (yield strength/break strength) of the steels is about 0.8 - 0.95.

It may be further concluded from the results of Tables 1 to 3 that the yield strength values of the steel strip in the machine direction and cross machine direction of the steel strip do not differ significantly from one another in examples 3, 4, 6, 7, 9, 11 and 12. The yield strength in the machine direction is almost as high as the yield strength in cross machine direction, the ratio of the strengths being < 6.5%, even < 2%. According to the examples, strength variations as low as these are obtained by carrying out the quenching according to a preferred embodiment of the invention to a temperature of less than 100°C and/or by using the final strip rolling temperature of 890°C.

As shown in Tables 2 and 3, said uniform quality is present in steels in which the final rolling temperature is low (below 890°C) and/or coiled at a low temperature (coiling temperatures 50°C).

Reference values from the table show for examples 1, 2a and 5 that when the coiling temperature is well over 100°C, the isotropy of the steel strength values decreases to a value closer to 10%, this representing a usual variation in strength values for a conventional, thermomechanically produced steel. The same applies to break strength values.

The effect of final bending temperature T_f and coiling temperature T_c on the isotropy of yield strength is examined in greater detail in Figures 6 and 7, which show that a decrease in both the final bending temperature and the coiling temperature allow the yield strength of the steel of the invention to be improved.

The invention has also shown that yield strength isotropy may be evaluated using formula Rp(T-L)/Rp(L) = - 46.6 + 0.0576 T_f + 0.0103 T_c, where T_f is the final bending temperature and T_c the coiling temperature.

Uniform quality is advantageous, because when a steel strip for different purposes is being designed, there is no need to take into account the fact that the steel strip has a higher strength in rolling direction than in the direction that is transverse to the rolling direction. Hence it is possible to take advantage of the high strength of the steel strip in all situations, i.e. also when cutting blanks that are processed into products which in use receive their greatest load in the direction that corresponds to the rolling direction of the steel strip. Further, the use of the steel strip may be optimized, because variations in strength in relation to the loading direction do not need to be taken into account. Moreover, isotropic strength properties probably contribute to the formation of bends of uniform quality irrespective of the bending direction (longitudinal/transverse), which further improves the applicability of the steel strip product of the invention. Table 4 shows that bendability in longitudinal bending, which is known to be problematic, is excellent. Steel sample B5Q3, for example, in longitudinal bending allows an R/t value of 1.3 to be reached. Transverse bending of this steel still succeeds at R/t value 0.3.

The bending has been carried out by a prior art method as a V-bend between the upper and the lower tool, Figure 3 illustrating the principle. The bending method used is free bending with a V-opening width V of 100 mm. The test pieces were bent in both directions, whereby they were bent into Z-shapes.

**Table 4. Bending results. Bending with a square sheet having a side length of 300 - 400 mm, and the bent made crosswise to the rolling direction. In the table R represents the bending radius and t the sheet thickness. The bending tests were made transversally (T) to the rolling direction.**

| | | **Bending results** | | |
|---|---|---|---|---|
| R/t | Direction | **Steel B3Q23 (bending test a) T=10mm** | **Steel B5Q23 (bending test c) T=6mm** | **Steel A3M33 (bending test b) T=10mm** |
| 2 | T | | OK | OK |
| 1.8 | T | | OK | |
| 1.6 | T | OK | | OK |
| 1.5 | T | | | |
| 1.4 | T | | | Fail |
| 1.25 | T | | OK | |
| 1.2 | T | OK | | Fail |
| 1 | T | OK | OK | Fail |
| 0.8 | T | OK | OK | Fail |
| 0.6 | T | OK | OK | Fail |
| 0.4 | T | OK | OK | Fail |
| 0.3 | T | | OK | |
| 2.2 | L | | OK | |
| 1.7 | L | | OK | |
| 1.3 | L | | OK | |
| 1 | L | | Fail | |
| 0.7 | L | | Fail | |

The results of the bending test have been analyzed visually. Figure 3 shows a successful bend (OK) with a round bend form and an intact surface. Rejecting result (Fail) is due to visible cracks, fissures or angularity in the area of the bending radius. Table 5 shows typical bending faults that lead to a rejecting result and Table 4 an example of a clearly failed bending (Fail).

**Table 5. Typical bending faults**

| Name | Description |
|---|---|
| Edge fracture | Edge fractures on shear edge of outer bend |
| Very thin surface fracture | Yield lines visible on the bend |
| Thin surface fracture | Yield lines show as distinct grooves |
| (Surface crack) | Possible crack on bend surface |
| Surface crack | Reflecting crack on bend surface |
| Open crack | Clear break on bend surface |

As shown in Figure 4, steel B3Q23 (bending test a in Table 2) has a far better bendability than steel A3M33 (bending test b in Table 2). In the steel of the invention the ratio of the bending radius to material strength (R/t) may be even 0.4, whereas the ratio achieved by conventionally manufactured reference steel is only about 1.6. The conclusion drawn from Tables 1 to 4 and Figure 5 is that the in the method of the invention direct quenching is performed to a temperature of 300°C at the most.

As shown in Table 3 and Figure 5, the impact strength values obtained for steel samples B4Q23 (transition curve d) are significantly better than those for steel samples A2M33 (transition curve c). The former steel samples have been direct quenched to a temperature of 50°C (cf. Table 2), whereas the latter have been cooled to a temperature of 615°C. Table 3 also shows that cooling to a high temperature of about 600°C (examples 1 and 10) results only in impact strength values that are typical for steel of this strength grade. As is shown, the impact strength of the steel of the invention at a temperature of -20°C is at least 200 J/cm² and/or at a temperature of -40°C at least 190 J/cm² and/or at a temperature of -60°C at least 180 J/cm².

Lastly, the invention will be illustrated by a more detailed description of test examples and the information in Tables 1 to 4.
Example 1. A strip rolling mill was used to roll a hot strip having a thickness of 5 mm and composition (A1) of Table 1. The roll parameters (A1M33) are shown in Table 2. The results (A1M33) are shown in Table 3. The results show that when the strip is coiled at a coiling temperature of 600°C, an excellent strength is achieved, but impact strength, however, remains on a normal level only. A noteworthy aspect is that yield strengths are clearly different in different testing directions, which is normal for micro-alloy steels conventionally rolled thermomechanically. Elongation level is normal.
Example 2. A strip rolling mill was used to roll a hot strip having a thickness of 5 mm and composition (A1) of Table 1. The roll parameters (A1M63) are shown in Table 2. The results are shown in Table 3. The results show that coiling at a relatively low coiling temperature (about 480°C) produces steel (A1M63) of a low strength but improved impact energy. Elongation level is normal. Cooling the strip to a still lower coiling temperature (about 250°C) increases the strength of steel (A1Q61) close to the normal level with clearly improved impact energy. Elongation remains below the normal level.
Example 3. A strip rolling mill was used to roll a hot strip having a thickness of 5 mm and composition (A1) of Table 1. The roll parameters (A1M83) are shown in Table 2. The results (A1M83) are shown in Table 3. The results show that coiling at a very low coiling temperature (about 50°C) raises strength to a good level close to normal with impact energy still clearly better than the normal level. Elongation remains below normal level.
Example 4. A strip rolling mill was used to roll a hot strip having a thickness of 8 mm and composition (B4) of Table 1. The roll parameters (B4Q23) are shown in Table 2 and the corresponding results in Table 3. The results show that coiling at a very low coiling temperature (about 50°C) increases strength to a normal level and provides an impact energy that is clearly better than normal. Again, it is noteworthy that yield strengths in the rolling direction are nearly the same both crosswise and lengthwise. Elongation is slightly below normal.
Example 5. A strip rolling mill was used to roll a hot strip having a thickness of 10 mm and composition (B2) of Table 1. The roll parameters (B2L13) are shown in Table 2, the corresponding results in Table 3. The results show that at a very high rolling temperature (910°C) and coiling at a coiling temperature of 360°C, yield strength lengthwise in the bending direction remains at a low level, but impact energy is still good. Elongation is approximately at a normal level.
Example 6. A strip rolling mill was used to roll a hot strip having a thickness of 10 mm and composition (B3) of Table 1. The roll parameters (B3Q25) are shown in Table 2, the corresponding results in Table 3. The results show that at a very low rolling temperature (about 800°C) and a very low coiling temperature (about 50°C) yield strength increases to a normal level also for a thick strip, with impact energy still on a good level. A noteworthy aspect is that yield strengths in relation to the rolling direction are the same both crosswise and lengthwise. Elongation is slightly below the normal level.
Example 7. A strip rolling mill was used to roll a hot strip having a thickness of 5 mm and composition (D1) of Table 1.The roll parameters (D1Q63) are shown in Table 2, the corresponding results in Table 3. The results show that reduction of alloying elements (Ti, Nb in particular) decrease strength heavily when the steel is rapidly cooled to a temperature of 50°C. Elongation and impact strength are at a good level.
Example 8. A strip rolling mill was used to roll a hot strip having a thickness of 7.7 mm and a composition (C1) of Table 1, the strip being then used for manufacturing a HF-welded quadratic tube beam with dimensions of 100mm x 250mm. The rolling parameters (C1Q35) are shown in Table 2 and the results measured from the tube beam in Table 3. The measured strength values are strengths obtained after the formation of the tube beams. Because of cold forming taking place in the manufacture of tube beams, impact strength values typically drop a little. The results show that the steel according to the method is well suited also for manufacturing high-strength tube beams.
Example 9. A strip rolling mill was used to roll a hot strip having a thickness of 8 mm and compositions (A3 and B4) of Table 1. The rolling parameters (A3M33 and B3Q23) are shown in Table 2 and the corresponding test results measured from the strip in Table 3. Table 4 shows a comparison of the bending of these steels (A3M33 and B3Q23), whereby it is noted that a direct quenched steel B3Q23 sustains bending well even at R/t value 0.4. Steel A3M33 cooled to a temperature of about 600°C can be successfully bent to R/t value 1.6.
Example 10. Figure 5 compares the impact strength values of steels A2M33 and B4Q23 at different testing temperatures by a Charpy V impact test. The compositions and manufacturing parameters of steels A2M33 and B4Q23 are shown in Tables 1 and 2. Direct quenched steel B4Q33 proves to be clearly better, maintaining its strength also at extremely low temperatures.
Example 11. A strip rolling mill was used to roll hot strip having thicknesses of 5 and 6mm and composition (E1) of Table 1. The rolling parameters (E1Q11 and E1Q33) are shown in Table 2 and the corresponding test results measured from the strip in Table 3. The results show that a steel strip product of the invention may be manufactured also in small thicknesses, for example by selecting the niobium, titan and vanadine contents of the steel as follows: Nb: 0.04 - 0.06%, Ti: 0.06 - 0.10% and V: 0.06 - 0.1%.
Example 12. A strip rolling mill was used to roll a hot strip having a thickness of 12 mm and compositions (F1 and F2) of Table 1. The rolling parameters (F1Q23 and F2Q43) are shown in Table 2 and the corresponding test results measured from the strip in Table 3. The results show that a steel strip product of the invention can be manufactured also with thick dimensions. In addition, this example further proves that uniform quality is obtained by direct quenching carried out to a temperature below 100°C and/or by using a strip rolling end temperature that is below 890°C.

In the above the invention has been illustrated by examples. On account of this it is to be noted that the details of the invention may be implemented in various ways within the scope of the accompanying claims.

## Claims

1. A method for manufacturing a hot-rolled steel strip product having a thickness of 2 to 12 mm by using steel whose composition in percentage by weight is
| | |
|---|---|
| C: | 0.04 - 0.08 |
| Si: | 0 - 0.5 |
| Mn: | 1.3 - 2.2 |
| Nb: | 0.04 - 0.09 |
| Ti: | 0.06 - 0.16 |
| N: | < 0.01 |
| P: | ≤ 0.03 |
| S: | < 0.015 |
| Al: | 0.01 - 0.15 |
| V: | ≤ 0.1 |
| Cr: | < 0.2 |
| Mo: | < 0.2 |
| Cu: | ≤ 0.5 |
| Ni: | ≤ 0.5 |
the rest consisting of iron and unavoidable impurities, **characterized by**
- austenizing a work piece of steel at an austenizing temperature of 1200 to 1350°C;
- hot rolling the steel work piece in a pre-rolling step;
- rolling the pre-rolled steel work piece in a strip rolling mill so that a rolling temperature of 760 to 960°C is achieved for the work piece in the last pass; and
- direct quenching the steel strip after the last pass in the strip rolling mill by a single-step cooling at a cooling rate of 30 to 150°C/s to 300°C at the most, the direct quenching being carried out within 15s from the last pass.

2. A method according to claim 1, **characterized in that** the end temperature of the direct quenching is 100°C at the most.

3. A method according to claim 1 or 2, **characterized in that** the steel strip is formed into a tube product after the direct quenching.

4. A hot-rolled steel strip product having a thickness of 2 - 12 mm and a composition in percentage by weight of
| | |
|---|---|
| C: | 0.04 - 0.08 |
| Si: | 0 - 0.5 |
| Mn: | 1.3- 2.2 |
| Nb: | 0.04 - 0.09 |
| Ti: | 0.06 - 0.16 |
| N: | < 0.01 |
| P: | ≤ 0.03 |
| S: | < 0.015 |
| Al: | 0.01 - 0.15 |
| V: | ≤ 0.1 |
| Cr: | < 0.2 |
| Mo: | < 0.2 |
| Cu: | ≤ 0.5 |
| Ni: | ≤ 0.5 |
the rest being iron and unavoidable impurities, **characterized in that** the microstructure of the steel is substantially low carbon ferritic and/or low carbon bainitic and contains high-carbon islands; that its yield strength is 650 - 800 MPa and percentage of elongation after fracture is at least 12%; and that its yield ratio is 0.8-0.95; and that its structure is isotropic in the sense that its yield strength in the rolling direction differs 6.5% at the most from its yield strength in the direction that is transverse to the rolling direction.

5. A steel strip product according to claim 4, **characterized in that** in crosswise bending the steel sustains a bending radius of 0.4 ≤ R ≤ 0.75 t, t being the wall thickness of the steel product, without cracks or fractures visible to the eye.

6. A steel strip product according to claims 4 or 5, **characterized in that** its average grain size is 2 to 4 micrometres.

7. A steel strip product according to any one of the preceding claims 4 to 6, **characterized in that** its carbon equivalent is 0.45 at the most.

8. A steel strip product according to any one of the preceding claims 4 to 7, **characterized in that** its yield strength is over 680 MPa.

9. A steel strip product according to any one of the preceding claims 4 to 8, **characterized in that** its impact strength at a temperature of - 20°C is at least 200 J/cm² and/or at a temperature of -40°C at least 190 J/cm² and/or at a temperature of -60°C at least 180 J/cm².

10. A steel strip product according to any one of the preceding claims 4 to 9, **characterized in that** it can be cut at a cutting gap of 10 - 15% of the sheet thickness without visually perceptible cracks.

11. A steel strip product according to claim 4, **characterized in that** the steel composition also meets the requirement Ti + Nb + V > 0.15.

12. A steel strip product according to claim 11, **characterized in that** its thickness is 2 - 6 mm and the contents of alloying elements Nb, Ti and V in the steel are
Nb: 0.04 - 0.06
Ti: 0.06 - 0.10
V: 0.06 - 0.10.

13. A steel strip product according to claim 10, **characterized in that** the molybdene content of the steel is Mo < 0.10.

14. A steel strip product according to claim 4 **characterized in that** its thickness exceeds 8 mm and that the copper and nickel content of the steel is 0.3 ≤ Cu ≤ 0.5 and Ni < 0.1%.

## Patentansprüche

1. Verfahren zur Herstellung eines warmgewalzten Stahlbandprodukts mit einer Dicke von 2 bis 12 mm unter Verwendung von Stahl, dessen Zusammensetzung in Gewichtsprozent ist :
| | |
|---|---|
| C: | 0,04 - 0,08 |
| Si: | 0 - 0,5 |
| Mn: | 1,3 - 2,2 |
| Nb: | 0,04 - 0,09 |
| Ti: | 0,06 - 0,16 |
| N: | < 0,01 |
| P: | ≤ 0,03 |
| S: | < 0,015 |
| Al: | 0,01 - 0,15 |
| V: | ≤ 0,1 |
| Cr: | < 0,2 |
| Mo: | < 0,2 |
| Cu: | ≤ 0,5 |
| Ni: | ≤ 0,5 |
wobei der Rest aus Eisen und unvermeidbaren Verunreinigungen besteht, gekennzeichnetdurch
- Austenitisieren eines Werkstücks aus Stahl bei einer Austenitisierungstemperatur von 1200 bis 1350°C;
- Warmwalzen des Stahlwerkstücks in einem Vorwalzschritt;
- Walzen des vorgewalzten Stahlwerkstücks in einem Bandwalzwerk, so dass im letzten Durchlauf für das Werkstück eine Walztemperatur von 760 bis 960°C erreicht wird; und
- direktes Abschrecken des Stahlbandes nach dem letzten Durchlauf im Bandwalzwerk durch Kühlen in einem Schritt mit einer Abkühlgeschwindigkeit von 30 bis 150°C/s bis höchstens 300°C, wobei das direkte Abschrecken innerhalb von 15 s nach dem letzten Durchlauf durchgeführt wird.

2. Verfahren nach Anspruch 1, **dadurch gekennzeichnet, dass** die Endtemperatur beim direkten Abschrecken höchstens 100°C beträgt.

3. Verfahren nach Anspruch 1 oder 2, **dadurch gekennzeichnet, dass** das Stahlband nach dem direkten Abschrecken zu einem Rohrprodukt geformt wird.

4. Warmgewalztes Stahlbandprodukt mit einer Dicke von 2 bis 12 mm und einer Zusammensetzung in Gewichtsprozent von
| | |
|---|---|
| C: | 0,04 - 0,08 |
| Si: | 0 - 0,5 |
| Mn: | 1,3 - 2,2 |
| Nb: | 0,04 - 0,09 |
| Ti: | 0,06 - 0,16 |
| N: | < 0,01 |
| P: | ≤ 0,03 |
| S: | < 0,015 |
| Al: | 0,01 - 0,15 |
| V: | ≤ 0,1 |
| Cr: | < 0,2 |
| Mo: | < 0,2 |
| Cu: | ≤ 0,5 |
| Ni: | ≤ 0,5 ; |
wobei der Rest Eisen und unvermeidbare Verunreinigungen sind, **dadurch gekennzeichnet, dass** die Mikrostruktur des Stahls im Wesentlichen kohlenstoffarmferritisch und/oder kohlenstoffarm-bainitisch ist und Inseln mit hohem Kohlenstoffgehalt enthält; die Dehngrenze 650 - 800 MPa beträgt und die Bruchdehnung mindestens 12% beträgt; und das Dehngrenzenverhältnis 0,8 bis 0,95 beträgt; und dass seine Struktur in dem Sinne isotrop ist, dass sich seine Dehngrenze in Walzrichtung höchstens um 6,5% von seiner Dehngrenze quer zur Walzrichtung unterscheidet.

5. Stahlbandprodukt nach Anspruch 4, **dadurch gekennzeichnet, dass** der Stahl beim Querbiegen ohne für das Auge sichtbare Risse oder Brüche einen Biegeradius von 0,4 ≤ R ≤ 0,75 t behält, wobei t die Wandstärke des Stahlprodukts ist.

6. Stahlbandprodukt nach den Ansprüchen 4 oder 5, **dadurch gekennzeichnet, dass** seine mittlere Korngröße 2 bis 4 Mikrometer beträgt.

7. Stahlbandprodukt nach einem der vorstehenden Ansprüche 4 bis 6, **dadurch gekennzeichnet, dass** sein Kohlenstoffäquivalent höchstens 0,45 beträgt.

8. Stahlbandprodukt nach einem der vorstehenden Ansprüche 4 bis 7, **dadurch gekennzeichnet, dass** seine Dehngrenze über 680 MPa beträgt.

9. Stahlbandprodukt nach einem der vorstehenden Ansprüche 4 bis 8, **dadurch gekennzeichnet, dass** seine Schlagfestigkeit bei einer Temperatur von -20°C mindestens 200 J/cm² und/oder bei einer Temperatur von -40°C mindestens 190 J/cm² und/oder bei einer Temperatur von -60°C mindestens 180 J/cm² beträgt.

10. Stahlbandprodukt nach einem der vorstehenden Ansprüche 4 bis 9, **dadurch gekennzeichnet, dass** es mit einem Schnittspalt von 10 - 15% der Blechdicke ohne sichtbare Risse geschnitten werden kann.

11. Stahlbandprodukt nach Anspruch 4, **dadurch gekennzeichnet, dass** die Stahlzusammensetzung auch die Anforderung Ti + Nb + V > 0,15 erfüllt.

12. Stahlbandprodukt nach Anspruch 11, **dadurch gekennzeichnet, dass** seine Dicke 2 - 6 mm beträgt und die Gehalte der Legierungselemente Nb, Ti und V im Stahl
| | |
|---|---|
| Nb: | 0,04 - 0,06 |
| Ti: | 0,06 - 0,10 |
| V: | 0,06 - 0,10 |
betragen.

13. Stahlbandprodukt nach Anspruch 10, **dadurch gekennzeichnet, dass** der Molybdängehalt des Stahls Mo < 0,10 beträgt.

14. Stahlbandprodukt nach Anspruch 4, **dadurch gekennzeichnet, dass** seine Dicke 8 mm überschreitet und das der Kupfer- und Nickelgehalt des Stahls 0,3 ≤ Cu ≤ 0,5 und Ni < 0,1% beträgt.

## Revendications

1. Procédé de fabrication d'un produit en bande d'acier laminé à chaud ayant une épaisseur de 2 à 12 mm en utilisant de l'acier dont la composition en pourcentage en poids est
| | |
|---|---|
| C: | 0,04 - 0,08 |
| Si: | 0 - 0,5 |
| Mn: | 1,3 - 2,2 |
| Nb: | 0,04 - 0,09 |
| Ti: | 0,06 - 0,16 |
| N: | < 0,01 |
| P: | ≤ 0,03 |
| S: | < 0,015 |
| Al: | 0,01 - 0,15 |
| V: | ≤ 0,1 |
| Cr: | < 0,2 |
| Mo: | < 0,2 |
| Cu: | ≤ 0,5 |
| Ni: | ≤ 0,5 |
le reste étant constitué de fer et d'impuretés inévitables, **caractérisé par**:
- austénisation d'une pièce à usiner d'acier à une température d'austénisation de 1200 à 1350°C ;
- laminage à chaud de la pièce à usiner en acier dans une étape de prélaminage ;
- laminage de la pièce à usiner d'acier pré-laminée dans un laminoir à bandes de manière à obtenir une température de laminage de 760 à 960 °C pour la pièce à usiner lors du dernier passage ; et
- trempe directe de la bande d'acier après le dernier passage dans le laminoir à bande par un refroidissement en une étape à une vitesse de refroidissement de 30 à 150 °C/s jusqu'à 300 °C au maximum, la trempe directe étant réalisée dans les 15 s à compter du dernier passage.

2. Procédé selon la revendication 1, **caractérisé en ce que** la température finale de la trempe directe est de 100 °C au maximum.

3. Procédé selon la revendication 1 ou 2, **caractérisé en ce que** la bande d'acier est transformée en un produit tubulaire après la trempe directe.

4. Produit en bande d'acier laminée à chaud ayant une épaisseur de 2 - 12 mm et une composition en pourcentage en poids de
| | |
|---|---|
| C: | 0,04 - 0,08 |
| Si: | 0 - 0,5 |
| Mn: | 1,3 - 2,2 |
| Nb: | 0,04 - 0,09 |
| Ti: | 0,06 - 0,16 |
| N: | < 0,01 |
| P: | ≤ 0,03 |
| S: | < 0,015 |
| Al: | 0,01 - 0,15 |
| V: | ≤ 0,1 |
| Cr: | < 0,2 |
| Mo: | < 0,2 |
| Cu: | ≤ 0,5 |
| Ni: | ≤ 0,5 |
le reste étant du fer et des impuretés inévitables, **caractérisé en ce que** la microstructure de l'acier est essentiellement ferritique à faible teneur en carbone et / ou bainitique à faible teneur en carbone et contient des îlots à haute teneur en carbone ; que sa limite d'élasticité est de 650 - 800 MPa et pourcentage d'allongement après fracture est d'au moins 12 % ; et que son taux de rendement est de 0,8 - 0,95 ; et que sa structure est isotrope en ce sens que sa limite d'élasticité dans la direction de laminage diffère au maximum de 6,5 % de sa limite d'élasticité dans la direction qui est transversale à la direction de laminage.

5. Produit en bande d'acier selon la revendication 4, **caractérisée en ce que**, lors de la flexion transversale, l'acier maintient un rayon de courbure de 0,4 ≤ R ≤ 0,75 t, t étant l'épaisseur de paroi du produit d'acier, sans fissures ni fractures visibles à l'oeil.

6. Produit en bande d'acier selon les revendications 4 ou 5, **caractérisée en ce que** sa taille de grain moyenne est de 2 à 4 micromètres.

7. Produit en bande d'acier selon l'une quelconque des revendications précédentes 4 à 6, **caractérisée en ce que** son équivalent en carbone est de 0,45 au maximum.

8. Produit en bande d'acier selon l'une quelconque des revendications précédentes 4 à 7, **caractérisée en ce que** sa limite d'élasticité est supérieure à 680 MPa.

9. Produit en bande d'acier selon l'une quelconque des revendications précédentes 4 à 8, **caractérisée en ce que** sa résistance au choc à une température de -20 °C est d'au moins 200 J/cm² et/ou à une température de -40 °C au moins de 190 J/cm² et/ou à une température de -60 °C au moins de 180 J/cm².

10. Produit en bande d'acier selon l'une quelconque des revendications précédentes 4 à 9, **caractérisée en ce qu'**il peut être coupé à un intervalle de coupe de 10 à 15 % de l'épaisseur de la feuille sans fissures perceptibles visuellement.

11. Produit en bande d'acier selon la revendication 4, **caractérisé en ce que** la composition d'acier répond également à l'exigence Ti + Nb + V > 0,15.

12. Produit en bande d'acier selon la revendication 11, **caractérisée en ce que** son épaisseur est de 2 - 6 mm et le contenu en éléments d'alliage Nb, Ti et V dans l'acier est
Nb: 0,04 - 0,06
Ti: 0,06 - 0,10
V: 0,06 - 0,10.

13. Produit en bande d'acier selon la revendication 10, **caractérisée en ce que** la teneur en molybdène de l'acier est Mo < 0,10.

14. Produit en bande d'acier selon la revendication 4, **caractérisée en ce que** son épaisseur est supérieure à 8 mm et que la teneur en cuivre et en nickel de l'acier est 0,3 ≤ Cu ≤ 0,5 et Ni < 0,1 %.
